

July 27, 1926.

1,593,598

K. REDMAN

METHOD OF DRYING MOISTURE CONTAINING MATERIALS

Filed Feb. 24, 1923

2 Sheets-Sheet 1



Inventor:

Fig. 2. Kenneth Redman  
Van Everen Fish Hildreth & Co  
Attn:

witness

Alfred H. McGehee

July 27, 1926.

1,593,598

K. REDMAN

METHOD OF DRYING MOISTURE CONTAINING MATERIALS

Filed Feb. 24, 1923

2 Sheets-Sheet 2



*Witness:*

Alfred H. McGlinchey.

*Inventor:*  
Kremette Redman  
by  
Van Ecorer, Fish, Heldreth & Cary  
Attny

Patented July 27, 1926.

1,593,598

# UNITED STATES PATENT OFFICE.

KENNETH REDMAN, OF WEST ROXBURY, MASSACHUSETTS, ASSIGNOR, BY MESNE ASSIGNMENTS, TO B. F. STURTEVANT COMPANY, OF BOSTON, MASSACHUSETTS, A CORPORATION OF MASSACHUSETTS.

## METHOD OF DRYING MOISTURE-CONTAINING MATERIALS.

Application filed February 24, 1923. Serial No. 621,059.

The present invention relates to a method of drying moisture-containing materials and is more particularly concerned with the kiln drying of lumber.

It has been appreciated by those skilled in the art for a considerable length of time that the drying of moisture-containing materials should be initiated in a relatively humid atmosphere in order that the drying action might be caused to take place gradually, thereby obviating the danger of cracking or warping of the drying material by drying the surface too rapidly. To this end, the older methods of drying lumber consist in merely subjecting the lumber to heated air or other gas at high relative humidity, this relative humidity being gradually decreased and the temperature being increased as the drying action progresses. This method, however, is rather slow, and accordingly possesses the disadvantage that long continued heating periods are required, thereby utilizing excessive amounts of fuel to say nothing of the charges involved in the long use of the kiln for one drying operation.

The principal object of the present invention is to provide a method of drying wood or other moisture-containing materials whereby the total drying operation may be much more rapidly performed with an increased quality of product.

Another object of the invention is to provide a method of drying moisture-containing material by which the entire drying operation may be more economically effected than in previous existing methods.

With these and other objects in view, the present invention consists of the method or steps hereinafter described and more particularly defined in the claims.

I have discovered that the drying of lumber or similar material may be greatly improved by alternately heating and cooling the lumber and providing after certain or each of the cooling periods an extended rest period during which the lumber is not subjected to currents of either hot or cold air. Accordingly, the principal feature of the present invention is the provision of the following cycle of operations in the drying of lumber: First, subjecting the lumber to a current of heated air or other gas of high humidity; second, passing a current of relatively cool air over the lumber; and third,

allowing the lumber to remain in a still atmosphere for a considerable length of time. The cycle of operations may then be repeated, it being preferable, however, to lower the relative humidity and increase the dry bulb temperature in the first step of the cycle.

It is believed that the advantages accruing to this method depend largely upon differences in vapor tension which may exist between moisture in the heated material and that of the surrounding air or gas and also to certain hygroscopic effects existing within the material. For example, the initial step of passing heated air of high relative humidity over the lumber thoroughly heats the lumber to a fairly high temperature and allows only partial drying of the wood, at the same time preventing excessive evaporation of the moisture from the surface. The vapor tension of the moisture at the surface or shell of the wood is thus made relatively high. The second step which consists in passing relatively cool air over the lumber allows evaporation of the moisture from the surface of the lumber into the current of air, due to the lower vapor tension of the moisture in the air. The draft of air may then be shut off and the lumber subjected to a rest period for a considerable length of time during which a transfusion of the moisture takes place from the central portion of the material to the outer surface, due to the fact that the central portion of the wood still retains its higher moisture content which tends to equalize with the surface of the lumber which has previously had its moisture content materially reduced during the preceding step. More moisture may then be removed from the wood by repeating the above cycle of operations as many times as may be desired. It has been found that this method of inserting a rest period into the cycle of operations not only reduces the operating time required for the kiln drying but produces an improved quality of product with greatly less liability of checking or otherwise injuring the lumber due to improper kiln operation. The method also possesses the advantage of requiring materially less heat and power for the entire operation.

Before applying any of the above steps, it is highly desirable, although not neces-

sary, that the material to be dried be heated throughout to a fairly high temperature but without any substantial drying. To this end, another feature of the invention provides for subjecting the material to a preliminary heating operation in the presence of an excess of moisture. This heating operation is conveniently carried out by injecting live steam directly into the kiln. 10 This preliminary step does not necessarily form a part of the repeated cycle of operations but is preferably carried out once only at the start of the drying operation. Certain other features of the invention 15 consist of certain novel features of construction and modes of operation hereinafter described and claimed, the advantages of which will be apparent to those skilled in the art from the following description. 20 In the accompanying drawings Figure 1 is a plan view in section of a fan type or forced draft kiln in which the improved method of the present invention may be carried out; Fig. 2 is a section on line 2—2 of Fig. 3 showing endwise piling of the lumber in the kiln; Fig. 3 is a sectional elevation of the kiln shown in Fig. 1; and Fig. 4 is a sectional elevation of a common form of pipe coil kiln showing crosswise piling of 30 the lumber.

The present invention resides in the cycle of operations and combinations of steps in the method of drying and the particular type of apparatus used may be of the usual 35 form with certain slight modifications which will hereinafter appear. The illustrated apparatus for carrying out the improved method comprises both forced draft kilns and pipe coil kilns with either of which the 40 method of the present invention may be employed.

Referring to Figs 1, 2 and 3, the forced draft kiln of the usual form consists of side walls 6, end walls 8, roof 10, floor 12 and suitable doors 14. The lumber is preferably piled 45 on trucks 16 and 18, the different layers of lumber being separated in the usual manner by stickers 20. In order that the air or gas may penetrate to all parts of the wood, the pile is preferably constructed with a central tapering flue 22, as indicated in Fig. 2. The trucks 16 and 18 are run into the kiln over rails 24. The circulation of air or other gas in the kiln is effected by a 50 fan or blower 26 having an inlet connected with heating coils 28 and a humidity sprayer 30, and an outlet connected with supply passages 32 and 34. The passages 32 and 34 communicate with supply ducts 36 and 38, respectively, which are tapering in form and are located beneath the trucks. The ducts are provided with louvers 40 and 42 of the usual form consisting of a series of upstanding metallic vanes. It will be seen that the 55 air passing through the fan is directed

through the passages 32 and 34 upwardly through the flues 22 by the louvers. A deflector 44 may be inserted at the joint between the passages 32 and 34 to control the flow of air in the passages 32 and 34 as desired.

The passage of the air through the kiln may be caused to take place by re-circulation or by the admission of fresh air from the atmosphere. To the former end, the air after passing through the flues 22 diverges from the lumber piles approximately as shown by the arrows in Fig. 2 and passes downwardly through openings 46 in the floor 12 into return ducts 48 which are connected at openings 49, and thence into an intake duct 50 leading directly to the inlet of the heater 28. In order to allow circulation of fresh air through the kiln, ventilators 52 and 54 are provided, the former leading directly to the inlet of the heater, as indicated in Fig. 1, and the latter being merely connected with an opening in the roof 10. The ventilator 52 is provided with a slide 56 and the ventilator 54 is provided with a damper 58 which may be actuated in any desired manner. Upon opening the slide 56 and damper 58 the circulation of fresh air from the atmosphere may be caused to take place within the kiln.

The humidity sprayer is fed with steam through a steam pipe 60 and a suitable valve 62. The steam pipe 60 also leads through a valve 64 to perforated steam pipes 66 and 68 resting upon the floor 12 for the purpose of injecting live steam into the kiln for the preliminary step of thoroughly heating the lumber.

The complete series of operations for drying lumber in the above desired type of kiln will now be enumerated in detail. The preliminary step consists of the admission of live steam to thoroughly heat the lumber through its mass. The average time for this operation is from two to four hours for one inch lumber and will, of course, vary with the thickness of the lumber and its previous degree of moisture. The first step in the cycle of operations consists in the admission of humid heated air into the kiln. To this end, the fan 26 is started and the valve 62 is opened to permit steam to be injected into the current of air through the humidity sprayer 30, the valve 64 being closed. In this step, it is desirable to approximate the humidity and temperature conditions recommended by the Forest Products Laboratory at Madison, Wisconsin, of the U. S. Government Department of Agriculture. The recommendations cover a considerable range of moisture content, thickness and kinds of lumber, and the humidity and temperature conditions may be readily adjusted to conform therewith. During this period it is desirable to re-circulate most of the air and

to this end the slide 56 and damper 58 should be slightly open during this step so that only 10% to 25% of the air re-circulated is continually refreshed. This heating and drying period is preferably continued for the remainder of the working day.

The second step of the cycle is comparatively short and consists in the rapid drying of water vapor from the surface or shell of the wood. To this end the humidity sprayer and heater coils are turned off and slide 56 and damper 58 are open wide to allow the circulation of fresh cool air through the kiln, continuing the operation of the fan 26 all the while. This step conveniently lasts from one to two hours. During this step the vapor tension of the moisture in the heated wood is much greater than that of the surrounding cooler air or gas. Since all pressures tend to equalize, it is believed that the vapor in the heated wood tends to create an equilibrium with the vapor tension in the cooler air. In so doing the surface moisture of the wood is rapidly given up, thereby cooling the wood until an equilibrium is reached, whereupon all moisture transfer to the atmosphere substantially ceases.

The third and final step in the cycle of operations consists of a rest period during which time the blower 26 is shut off. Communication with the atmosphere is maintained by keeping the ventilators open but no forced circulation of air is necessary. During this period, it is believed that due to the hygroscopic character of the wood, the moisture contained in the central portions tends to establish an equilibrium with the surface or shell which has just been dried during the second step of the cycle above described. That is to say, the surface or shell absorbs moisture from the center so that at the conclusion of the rest period, the surface again contains moisture which may be readily evaporated by repetition of the preceding cycle. This rest period preferably continues over a number of hours and accordingly may last all night. It will be seen that the use of heat and power during the night is thus obviated and furthermore, no attention is required.

Upon arrival of the workman in the morning, the kiln is once again started preferably omitting, however, the preliminary steaming operation. The heating step with humid air is carried through this time, however, with a reduced relative humidity and an increased dry bulb temperature. This is followed, as before with the drying by means of cool air delivered by the fan, and this in turn by the rest period. The cycle of these three steps may be repeated as many times as desired, the temperature preferably being increased, and the humidity decreased with each recurrence of the first step.

It is believed that the foregoing remarks

correctly explain the theoretical operation of the improved method. Regardless of the correctness of this theory, however, it is known that this method produces a higher quality of product than previously existing methods and may be much more economically carried out.

A slight modification of the above procedure may be carried out with thin lumber or veneer. In this case the passage of the moisture from the internal to the external layers does not require considerable lengths of time so that in the first cycle of operations the extended rest period may be considerably reduced or, in fact, omitted altogether. During the second cycle, however, the rest period should be used for maximum economy and rapidity of drying.

The features of the present invention are not alone applicable to the forced draft type of kiln but may be embodied in a pipe coil kiln of the usual form. In this type of kiln, the heating is done by convectional currents of air which are heated over a series of pipes containing steam or other heating fluid. Referring particularly to Fig. 4, the pipe kiln is constructed with side walls 6 and roof 10, as before. The trucks 16 are preferably run in over three rails 24 if the illustrated form of crosswise piling is employed. As before, the successive layers of lumber are separated by stickers 20. Fresh air is admitted to the kiln through air ducts 70 and is allowed to pass over the rows of heated pipes 72. The air is raised to the proper humidity by steam from the perforated steam pipes 66 and 68 and then passes up through the lumber. The pipes 66 and 68 are used both for the preliminary steaming operation and for humidifying the entering air. After passing upward through the lumber pile the currents of air diverge and pass outwardly to the atmosphere through dampers 74 inserted in ventilators 76 and 78.

For this type of kiln the steps are carried out approximately as in the forced draft type of kiln. The preliminary steaming operation is effected by closing the air ducts 70 and the dampers 74 and turning on the steam in pipes 66 and 68 for a period of two to four hours. The first heating step in the cycle is then carried out as in the case of the forced draft kiln. The pipes 72 are heated by the passage of steam therethrough and the ducts 70 and dampers 74 are opened to allow the circulation of heated air upwardly through the lumber pile, the proper humidity being maintained by regulation of the steam in pipes 66 and 68. As in the previous case, this operation is carried out for the remainder of the working day. The temperature and humidity may be substantially the same as in the other case but it is desirable to have the temperature slightly higher

and the humidity somewhat lower to compensate for the slower circulation. The second step in the cycle consists, as before, in passing the cool dry air over the lumber. 5 This is caused to take place by natural instead of forced circulation. The previously heated condition of the lumber and kiln building will tend to permit circulation of the air therethrough. The steam in pipes 10 66 and 68 is turned off during this step. As in the previous case, the third and final step consists in a rest period during which time a transfusion of the moisture occurs from the central portions of the wood to the surface. 15 In the case of a pipe coil kiln, this rest period obtains as soon as the vapor tension of the moisture in the wood substantially equalizes with the vapor tension of the surrounding air or gas, that is, when 20 the temperatures of the lumber and gas have become practically equalized. During this rest period there is substantially no circulation of air through the kiln. It is to be pointed out that as in the case of the forced 25 draft kiln, the several steps are separate and distinct and although the line of demarcation between the second and third steps may not be as pronounced in the pipe coil kiln as in the forced draft kiln, there is nevertheless 30 no difference in the principle of operation between the two types of kilns as in both types the second step consists in the evaporation of moisture from the surface of the wood and the third step consists in the 35 transfusion of the moisture from the interior to the shell of the wood. The only difference is that in the case of the pipe coil kiln, the change from the second to the third step is gradual and takes place naturally due 40 to the equalization of the temperatures rather than through any actual operation of the apparatus as in the case of the forced draft kiln. After the completion of the rest period, the cycle of operations is carried on 45 as before, preferably omitting the preliminary steaming operation.

Although the present invention has been specifically described in connection with the drying of lumber, it is understood that the 50 invention should not be so limited, but should extend to the drying of other materials. The invention should also not be considered limited to the specific steps described herein except as limited in scope 55 by the appended claims.

The invention having been described, what is claimed is:—

1. The method of drying moisture-containing materials which consists in subjecting the material to a current of heated air or gas at high relative humidity, then to a current of materially cooler gas, allowing the material to rest for a period sufficient to permit diffusion of the moisture from the 60 central portion to the surface of the mate- 65

rial, and thereafter subjecting the material to a current of heated air.

2. The method of drying materials which consists in subjecting the material to the following cycle of operations; first, passing a current of heated air of high relative humidity over the material; second, cooling the material by a current of air at materially lower temperature to allow vaporization at the surface of the material by differences 75 in vapor tension between the moisture at the surface of the material and the moisture in the air; third, allowing the material to rest without further drying action for a period sufficient to permit transfusion of the moisture outwardly from the central portion of the material; and fourth, passing a current of air over the material to absorb moisture 80 from the surface thereof.

3. The method of drying materials which 85 consists in repeatedly and alternately passing heated air of high relative humidity and materially cooler air over the material and allowing the material to rest without further drying after certain of the cooling 90 periods to permit transfusion of moisture outwardly from the central portions of the material.

4. A method of drying materials which 95 consists in thoroughly heating the material throughout its mass without drying and thereafter subjecting it to the following repeated cycle of operations; first, subjecting the material to a circulation of humid heated air, then passing a current of relatively 100 dry air at a lower temperature over the material to permit differences in vapor tension to cause evaporation of moisture from the surface of the lumber, and thereafter allowing the lumber to rest without further drying action for an extended period to permit 105 transfusion of moisture outwardly from the central portions of the material.

5. The method of kiln drying lumber which 110 consists in thoroughly heating the lumber throughout its mass by contact with steam, then repeatedly passing alternate currents of heated humid air and relatively dry air at a lower temperature over the lumber, and thereafter allowing the lumber to rest without 115 drying action at the conclusion of certain of the cooling periods for extended periods to permit transfusion of moisture from the central portion toward the surface of the lumber.

6. The method of drying moisture-containing materials which consists in subjecting the material to a current of heated air or gas at high relative humidity, then to a current of materially cooler gas until the 125 material attains substantially the temperature of the cooler gas, and thereafter allowing the cooled material to remain in the cooler gas to permit the diffusion of moisture 130 from the central portion to the surface of

the material, and then again subjecting the material to a current of heated air or gas and thereafter to a current of cooler gas.

7. The method of drying materials which consists in heating the material and drying, then cooling the same by subjecting it to a current of cool air, then permitting the cooled material to stand without drying, and thereafter again heating and drying the material.

8. The method of drying moisture-con-

taining materials which consists in subjecting the material to a current of heated air or gas at high relative humidity, then to a current of materially cooler gas, thereafter allowing the material to remain in the cooler gas and then again subjecting the material to a current of heated air or gas but of higher temperature and lower humidity than the former current of heated air. 15

KENNETH REDMAN.